

# UNITED STATES PATENT OFFICE

CLEMENT L. PERKINS AND RALPH E. SAYRE, OF PITTSBURGH, PENNSYLVANIA,  
ASSIGNORS TO METALS RECOVERY COMPANY, OF NEW YORK, N. Y., A CORPO-  
RATION OF MAINE.

## FLOTATION OF MINERALS.

1,364,307.

Specification of Letters Patent.

Patented Jan. 4, 1921.

No Drawing.

Application filed November 11, 1919. Serial No. 337,322.

To all whom it may concern:

Be it known that we, CLEMENT L. PERKINS and RALPH E. SAYRE, citizens of the United States, residing at Pittsburgh, Allegheny county, State of Pennsylvania, have invented certain new and useful Improvements in Flotation of Minerals; and we do hereby declare the following to be a full, clear, and exact description of the invention, such as will enable others skilled in the art to which it appertains to make and use the same.

This invention relates to the concentration of minerals, such as sulfid ores and the like, by flotation, and is based upon the discovery that improved results can be obtained by carrying out the flotation operation with the addition to the ore or mineral pulp of organic compounds containing sulfur and nitrogen, particularly sulfur derivatives of compounds containing reduced nitrogen. Organic sulfur-nitrogen compounds which have been found effective in the flotation of minerals include thio-ureas, thio-cyanogen compounds, thio-amido compounds or sulfur derivatives of amines, amido-thiophenols, as well as certain other compounds belonging to other groups.

Among the organic nitrogen-sulfur compounds which can thus be used may be mentioned the following:

Diphenyl-thiourea, (thio carbanilid,) Monophenyl-thiourea,  
Di-o-tolyl-thiourea,  
Di-p-tolyl-thiourea,  
Di-xylyl-thiourea,  
Phenyl-iso-thiocyanate,  
Thioanilin, (p-diamido-diphenyl sulfid,) Dehydro-thio-p-toluidin,  
Dehydro-thio-o-toluidin,  
Dithio-diphenyl amine,  
Diphenyl-thio-carbazid,  
Thiuram-disulfid,  
Thialdin,  
Carbothialdin,  
Amino-thio-phenol,  
Diamino-phenyl-disulfid.

These various organic substances all contain nitrogen and sulfur. Their methods of preparation are known and need no detailed description. However, the compounds need not, in many cases, be isolated in a state of purity but may be used in an impure state or accompanied with such by-products as are

formed at the same time. Thus, for example, where the thio compounds of amines or of other nitrogen compounds are produced by heating the nitrogen compounds with sulfur and where the resulting reaction mixture is liquid, the mixture itself may be used directly in flotation without isolation of the sulfur-nitrogen compounds as such in a state of purity. The compound thus produced may in fact be accompanied by by-products or by unchanged nitrogenous compounds which act as a solvent for the compounds produced or which themselves contribute to the value of the product in the flotation process. An effective flotation agent may thus be made by boiling toluidin with sulfur and the resulting product may be used, without further purification, in the flotation process.

The valuable properties of many, if not all, of the organic nitrogen-sulfur compounds above referred to appears to be related to the fact that these compounds are in a reduced state rather than in an oxidized state.

In carrying out the flotation process, the flotation agent or agents may be incorporated with the ore or mineral pulp in any suitable manner, for example, by introduction into the tube mill in which the ore is being ground, or by mixing or digesting with water and adding the resulting product to the ore pulp just before it enters the flotation apparatus, or by dissolving the flotation agent (where it is not itself readily incorporated with the mineral pulp) in an organic solvent therefor, or in one of the usual flotation oils or oil mixtures, and incorporating the resulting solution with the ore pulp, or in other suitable manner which will insure the uniform dissemination of the flotation agent throughout the pulp.

Certain of the flotation agents above referred to have been found to have a marked action as collecting or mineral modifying agents, even where they have little, if any, frothing qualities. In such cases they can be used to advantage in conjunction with other flotation agents which have good frothing qualities.

After the flotation agent or agents have been thoroughly and uniformly distributed throughout the ore pulp, the resulting mixture is subjected to a flotation operation, as

in an ordinary Callow cell or other pneumatic flotation cell, or in apparatus where the air is incorporated in the ore pulp by mechanical agitation.

5 The action of the flotation agents above referred to is sufficiently marked so that but a small amount thereof will usually be required, for example, with many of these agents, as little as one-fifth of a pound per 10 ton of ore, although in some cases even smaller amounts may be used, as well as materially larger amounts. When used in conjunction with other agents which have good frothing qualities, a fraction of a pound of 15 each agent per ton of ore will usually suffice.

We have also found that the flotation process can be improved, with certain ores, and with certain of the agents above specified, for example, with copper sulfid ore (of the Utah Copper Company) by the addition of alkali, such as sodium hydroxid or lime, which can be incorporated with the ore pulp in any suitable manner, as by grinding 25 therewith in the usual mill. The amount of alkali may be, for example, two pounds of caustic soda per ton of ore.

The invention will be further illustrated by the following specific example of a test 30 made upon a so-called porphyry ore of the Utah Copper Company which is a copper sulfid ore having a silicious gangue and containing its floatable or sulfid copper in the form of a mixture of chalcocite and chalco- 35 pyrite. In general, treatment of the ore with alkalis, as above noted, gives improved results, the alkalis themselves apparently having a valuable effect in improving the flotation process.

40 Five hundred parts by weight of the ore was ground in a pebble mill with two hundred and fifty parts of water, sodium hydroxid equivalent to two pounds per ton of dry ore, and dehydro-thio-p-toluidin equivalent to one-fifth pound per ton. The ground pulp was then transferred to a Callow rougher cell and subjected to flotation with the addition of about one-tenth pound of terpineol per ton. Terpineol pro- 45

50 duces a relatively voluminous froth but has very little tendency to float the sulfid in the ore when used by itself. The heads from this test contained 1.39% copper; the concentrate produced contained about 23% 55 copper; and the recovery was about 74.5%.

Better recoveries have been obtained with somewhat larger amounts of dehydro-thio-p-toluidin, for example, one test using one pound per ton gave a 16.4% concentrate and 60 87.3% recovery.

In the above example, lime, in the same or somewhat larger proportions, may be substituted for sodium hydroxid. So also, other suitable frothing agents may be substituted for the terpineol. 65

Dehydro-thio-p-toluidin is one of the sulfur derivatives of amines. It may be made by prolonged heating of p-toluidin with sulfur. It is a crystalline solid and is commonly regarded as insoluble. It may be advantageously incorporated with the ore pulp by adding the finely powdered dry compound to the ore pulp in the grinding mill. It may also be dissolved in appropriate organic solvents therefor, particularly those which have good frothing qualities and which will contribute to the carrying out of the flotation operation, for example, xylidin, or other suitable amines. 75

In our companion application Serial No. 284,981, filed March 25, 1919, we have described and claimed the improved flotation process in which thio-urea compounds or substances, and specifically thio-carbanilid, are employed, and such process accordingly is not claimed specifically herein, although it is included within the more comprehensive claims appended hereto, but the more specific claims of the present case are directed to the process in which thio-amido compounds, and specifically dehydro-thio-p-toluidin, are employed. So also, while certain of the organic nitrogen-sulfur compounds above referred to are substantially non-frothing collecting or mineral modifying agents, no claim is made herein to the process in which such agents generally are employed, inasmuch as such process forms the subject matter of an application of one of us, (Perkins) Serial No. 312,247 filed July 21, 1919; but the claims of the present case are directed to the process in which organic nitrogen-sulfur compounds of the character above described are employed, irrespective of whether such compounds are substantially non-frothing, or have frothing, as well as mineral modifying properties. The process of the present invention is also distinguished from the process in which salts of amido compounds are employed, such as sulfates, which contain sulfur in the acid radical of the salts, as set forth in the application of one of us, (Perkins) Serial No. 308,261 filed July 2, 1919. 90 95 100 105 110 115

The process of the present invention can be carried out in combination with the use of many of the usual oil mixtures which are commonly employed in flotation, by the addition of small amounts of one or more of the agents above referred to. Flotation oils or oil mixtures which have good frothing qualities, such as pine oil and other wood distillation oils, are of particular value inasmuch as they supplement the action of the organic nitrogen-sulfur compounds and are themselves supplemented in their action by such compounds. 120 125

The action of many of the organic nitrogen-sulfur compounds in the flotation process appears to be a selective action upon the 130

mineral surfaces rather than any action of importance upon the water itself. The modifying action of the collecting agents upon the mineral particles is sufficiently marked so that it is possible to raise relatively large mineral particles and hence fine grinding becomes of less importance.

We claim:

1. The method of effecting the concentration of minerals by flotation, which comprises adding to the mineral pulp a small amount of an organic nitrogen-sulfur compound, and subjecting the resulting mixture to a flotation operation; substantially as described.

2. The method of effecting the concentration of minerals by flotation, which comprises adding to the mineral pulp a small amount of a sulfur derivative of a compound containing reduced nitrogen, and subjecting the resulting mixture to a flotation operation; substantially as described.

3. The method of effecting the concentration of minerals by flotation, which comprises adding to the mineral pulp a small amount of an organic thio-amido compound, and subjecting the resulting mixture to a flotation operation; substantially as described.

30 4. The method of effecting the concentration of minerals by flotation, which comprises adding to the mineral pulp a small amount of dehydro-thio-p-toluidin, and subjecting the resulting mixture to a flotation operation; substantially as described.

35 5. The method of effecting the concentration of minerals by flotation, which comprises adding to the mineral pulp a small amount of an organic nitrogen-sulfur compound, together with an agent having good frothing qualities, and subjecting the resulting mixture to a flotation operation; substantially as described.

40 6. The method of effecting the concentration of minerals by flotation, which comprises adding to the mineral pulp a small amount of a sulfur derivative of an organic compound containing reduced nitrogen, together with an agent having good frothing qualities, and subjecting the resulting mixture to a flotation operation; substantially as described.

45 7. The method of effecting the concentration of minerals by flotation, which comprises adding to the mineral pulp a small amount of an organic thio-amido compound, together with an agent having good frothing qualities, and subjecting the resulting mixture to a flotation operation; substantially as described.

50 8. The method of effecting the concentration of minerals by flotation, which comprises adding to the mineral pulp a small amount of dehydro-thio-p-toluidin, together with an agent having good frothing

qualities, and subjecting the resulting mixture to a flotation operation; substantially as described.

9. The method of effecting the concentration of minerals by flotation, which comprises adding to the mineral pulp a small amount of an organic nitrogen-sulfur compound in an organic solvent therefor, and subjecting the resulting mixture to a flotation operation; substantially as described.

75 10. The method of effecting the concentration of minerals by flotation, which comprises adding to the mineral pulp a small amount of an organic nitrogen-sulfur compound, together with a small amount of alkali, and subjecting the resulting mixture to a flotation operation; substantially as described.

80 11. The method of effecting the concentration of minerals by flotation, which comprises adding to the mineral pulp a small amount of an organic nitrogen-sulfur compound, together with a small amount of alkali and an agent having good frothing qualities, and subjecting the resulting mixture to a flotation operation; substantially as described.

85 12. The method of effecting the concentration of minerals by flotation, which comprises adding to the mineral pulp a small amount of a sulfur derivative of an organic compound containing reduced nitrogen together with a small amount of alkali, and subjecting the resulting mixture to a flotation operation; substantially as described.

90 13. The method of effecting the concentration of minerals by flotation, which comprises adding to the mineral pulp a small amount of a sulfur derivative of an organic compound containing reduced nitrogen together with a small amount of alkali and an agent having good frothing qualities; and subjecting the resulting mixture to a flotation operation; substantially as described.

95 14. The method of effecting the concentration of minerals by flotation, which comprises adding to the mineral pulp a small amount of a sulfur derivative of an organic amido compound, together with a small amount of alkali and of an agent having good frothing qualities, and subjecting the resulting mixture to a flotation operation; substantially as described.

100 15. The method of effecting the concentration of minerals by flotation, which comprises adding to the mineral pulp a small amount of dehydro-thio-p-toluidin, together with a small amount of alkali and of an agent having good frothing qualities, and subjecting the resulting mixture to a flotation operation; substantially as described.

In testimony whereof we affix our signatures.

CLEMENT L. PERKINS.  
RALPH E. SAYRE.